

## UNITED STATES PATENT OFFICE

ARTHUR W. BURWELL, OF NIAGARA FALLS, NEW YORK, ASSIGNOR TO ALOX CHEMICAL CORPORATION, OF NEW YORK, N. Y., A CORPORATION OF NEW YORK

## LUBRICANT AND PROCESS OF MAKING THE SAME

No Drawing.

Application filed December 18, 1928. Serial No. 326,901.

The present invention relates to a method of increasing the lubricity of oils,—particularly, of oils of mineral origin,—and to lubricating compositions produced thereby.

5 It heretofore has been recognized that the lubricating powers of oils such as petroleum lubricating oils may be improved by incorporating therein or commingling therewith certain modifying agents, such, for example, 10 as free fatty acids or their corresponding water-insoluble, or water-soluble soaps, or naturally occurring fatty oils such as lard oil, neat's-foot oil, tallow, wool fat, and the like.

15 I now have prepared new and valuable lubricating oil compositions consisting essentially of mixtures of known lubricating oils of petroleum origin with addition materials (which will be described hereinafter with 20 greater particularity) consisting of certain high-molecular-weight, oxygen-containing, saturated aliphatic compounds, resulting from the controlled oxidation of aliphatic hydrocarbons of mineral origin as described 25 generally in my U. S. Patents Nos. 1,690,768 and 1,690,769. I have found that any one of such compositions possesses a markedly increased lubricity (i. e., greater capacity to lubricate) over that of an equal amount of 30 the known lubricating oil which forms the major component of said composition. Furthermore, there is experienced no corrosion of metal surfaces "wetted" by the compositions; in fact, distinct anti-rusting properties 35 obtain.

These "addition materials" exert no gumming effect either of themselves or in the compositions, nor do they oxidize upon continued exposure to air. The said materials 40 not only are relatively inexpensive (as compared with agents heretofore proposed) but also are economical in that relatively smaller proportions thereof are used.

In my United States Patents Nos. 1,690, 45 768 and 1,690,769, I have described generally a process of making aliphatic acidic compounds by controlled oxidation of hydrocarbons or mixtures thereof such as the hydrocarbons occurring in or associated with petroleum oils, in liquid phase, at a tempera-

ture above 100° C. but not substantially above 150° C., and at a pressure greater than atmospheric pressure but not substantially above about 320 pounds per square inch, in the presence of an exciter of oxidation, agitation and the necessary oxygen supply being furnished by passing a stream of free oxygen containing gas (e. g. air) through the body of hydrocarbons undergoing treatment.

By the expression "an exciter of oxidation" I mean to include the known oxidation catalysts such as, for example, manganese stearate and other catalytically acting compounds of manganese or copper or iron, known oxygen carriers, and especially hereinafter-mentioned unsaponifiable, non-acidic, components of a previously oxidized body of hydrocarbons. In my co-pending application Serial No. 156,053, filed December 20, 1926, it has been noted that a petroleum hydrocarbon mixture comprising in part the material which has already been subjected to the treatment does not require the presence of an oxidizing catalyst or of added exciter of oxidation in order to effect normal oxidation.

During the course of such an oxidizing treatment, small amounts of volatile acids (typified by formic acid), volatile ketones and other low molecular weight products are 80 formed, and are separated from the liquid undergoing treatment as vapors, along with carbon dioxide and, where air has been used as the oxidizing medium, air freed from substantially all of its normal content of oxygen.

At a comparatively early stage of the oxidation there begin to be formed ketones, alcohols, and acidic compounds having the structure of saturated aliphatic carboxylic acids,—all of relatively high molecular 90 weight. These acidic compounds are insoluble in water but soluble in petroleum hydrocarbons and in the reaction mixture.

By protraction of the oxidation treatment 95 it is possible to produce in the reaction mixture compounds which are insoluble in petroleum hydrocarbons and in the reaction mixture, which latter compounds have the nature of saturated, aliphatic, hydroxy-car-

boxylic acids and apparently result from an alternation of one or more



5 groups of the aliphatic chain to



12 groups.

13 According to the present invention I operate in the above manner upon relatively high molecular-weight aliphatic hydrocarbons of mineral origin, including the petroleum-type waxes obtainable from oil shales and from other bituminous materials including brown coals, but preferably petroleum waxes (e. g. rod wax, scale wax, the so-called "Sharples wax", and the like) and such petroleum distillates as consist chiefly 15 of relatively high molecular weight hydrocarbons. Since the product forming the basis of the present invention is derived from the said acidic compounds which are insoluble in water but soluble in petroleum hydrocarbons and in the reaction mixture, and since the 20 yield of said petroleum-soluble acidic compounds may be depreciated by protracted oxidation, by the conversion of a portion thereof to petroleum-insoluble acidic compounds, I prefer, for economic reasons, not to protract the oxidation treatment beyond 25 the point of incipient formation of the above-described petroleum-insoluble compounds.

30 Incipient formation of petroleum-insoluble compounds in the reaction mixture may be noted by simple observation of a test sample taken from the mixture, or by titration of such a sample. The time period is a handy, but not necessarily exact, indication of the 35 stage of the oxidation. In those cases where the reaction mixture does contain an appreciable or material amount of the said petroleum-insoluble acidic compounds, the latter may be separated from the reaction mixture by the method set out in lines 122 to 128, page 2 of my U. S. Patent No. 1,690,769, consisting in treating said mixture with petroleum distillate.—such, for example, as the 40 oil whose lubricating properties it is intended to improve by the addition thereto of the acidic compound,—and removing therefrom the resulting insoluble residue.

45 The resulting reaction mixture then is subjected to treatment with a hot aqueous solution of a caustic alkali whereby to saponify as completely as possible all the saponifiable compounds contained therein. Unsaponifiable components of the reaction mixture collect—by gravity separation—as a supernatant oily layer above a subnatant layer of 50 soap solution. Either of the two layers may be separately removed from their mutual container: e. g., the oil layer may be decanted, or the aqueous layer may be drawn off from 55 below. The resulting soap solution is sepa-

rated from the unsaponifiable constituents of the reaction mixture, the soap solution being further subjected to clearing by careful dilution with water until no more compounds are thrown out of solution and the main amount 60 of soap solution becomes clear. It is from this soap solution that my "addition materials" are derived.

65 The soap solution, after separation from any compounds thrown out of solution by reason of the dilution, is acidified as for instance with a mineral acid, whereby to liberate those compounds which were united with the alkali. There will be found to be present in the mass precipitated by this reaction 70 practically all, or at least the major portion, of the formed water-insoluble acidic compounds which are mono-carboxylic in their nature.

75 This precipitated mass then is transferred to a still where it is subjected to a very careful steam distillation; i. e., brought to and maintained at a point somewhat above the boiling point of water, and treated by passing therethrough a vigorous current of steam 80 until substantially no more volatile material passes over and until the odor of the mass has been so modified as to be no longer disagreeable. The resulting still residue, after 85 careful drying, is my "addition material", and is in a condition suitable for direct admixture with the lubricating oil.

90 The same practical result may be obtained by substituting an extraction procedure for the saponification and acidification procedure above described. As extractant there 95 may be used ethyl alcohol, acetone or like ketone, or a higher alcohol. I have found ordinary 95% alcohol to be a desirable solvent for the "saponifiable portion" of the 100 reaction mixture, and to have the effect of separating from the reaction mixture essentially the same mass or composition as is separated by practicing the saponification and acidification procedure above described. 105 The extraction preferably (although not necessarily) is carried out at such a temperature as insures maintaining the components of the reaction mixture in liquid state. It 110 is to be understood that by the expression 115 "separating the saponifiable components from at least the major portion of the unsaponifiable components" appearing in certain of the appended claims I mean to refer to either of the two optional separation procedures just described.

120 The aforesaid mass, upon examination is found to consist of from about 50% to about 75% of the hereinbefore mentioned acidic compounds and from about 50% to about 125 25% of unsaponifiable ketonic, alcoholic, and keto-alcoholic compounds,—all of relatively high molecular weight, which are miscible with the acidic compounds. Incidentally it is noted that these unsaponifiable oxygen- 130

containing compounds persist in accompanying the said soap solutions,—even in clear solution in any dilution. It is possible to separate them substantially completely from 5 the mass only by thorough extraction with ether or other equivalent organic solvent.

The said unsaponifiable compounds not only do not detract from the lubricity-increasing properties of the "addition materials" but exert a beneficial influence of the order of that of the acidic-compounds components of said "addition materials". The addition materials vary somewhat as to the relative proportions of their components, de- 10 pending in part upon the starting material selected, and in part upon the desired characteristics of the lubricating oil compositions to be produced. Typical analyses show the following compositions:

|    |                                                                                                                        |            |             |
|----|------------------------------------------------------------------------------------------------------------------------|------------|-------------|
| 20 | Free acids which will liberate carbon dioxide from cold aqueous solutions of sodium or potassium carbonate             | 23% to 40% | Average 30% |
|    | Lactones                                                                                                               | 3% to 25%  | 17%         |
|    | Combined acids as esters (not lactones)                                                                                | 4% to 25%  | 18%         |
| 25 | Unsaponifiable matter consisting almost exclusively of alcohols, alcohol-ketones or ketones, or a mixture of all three | 25% to 40% | 35%         |

The said addition materials, so prepared, are readily soluble in or miscible with lubricating oils, and the preparation of admixtures requires no especial instruction. While they do no harm to the metals with which they come into contact, and therefore can be used in lubricating oil compositions in considerable amounts,—say, 2.5% to 10% by weight, or higher,—I prefer, for reasons of economy, to use much smaller amounts since I find that additions of the order of from about 0.25 to about 0.75% by weight effect 30 astonishing results in breaking the surface tension of oils used on moving parts and in causing the oils to "wet", and cling to, metal surfaces. Compositions containing my addition materials in the latter content range 35 (i. e., 0.25%–0.75%) appear to give an improvement in lubricity equivalent to that effected by from 3% to 5% by weight of certain previously used fatty oils. Larger additions appear not to materially increase this effect. Furthermore, my new addition materials appear to assist in breaking down the 40 internal friction of lubricating oils.

As an instance of the above on the same bearing over a long period of time, the following results of tests are noted: A given lubricating oil of petroleum origin, during the course of a protracted test, showed a given rise in temperature. Upon the addition of 0.50% by weight of my addition material to another portion of the same oil and the substitution of the resulting composition for the "straight" lubricating oil under exactly the same conditions of room temperature, load, speed of shafting, etc., the temperature 45 did not rise to the same given point by as

much as 35° C. As the result of a series of such investigations with various lubricating oils, it was found that the temperature decrease upon addition of my addition material ranged from 16° to 35° C., with an average decrease of about 22° C. 70

The invention has been described with particular reference to the use of my "addition materials" in lubricating oil compositions adapted for use between moving parts (i. e., as engine oil, bearing oil, and the like). It should be noted that the use of said "addition materials" is not restricted thereto, but includes admixture with known "mold oils" 75 as excellent compositions for oiling the surfaces of metallic molds, such, for example, as those in which are cast objects of concrete, gypsum, basic magnesium chloride and the like, and that the hereinafter claims are intended to protect my novel addition materials per se, and as well lubricating oil compositions containing said addition materials irrespective of their particular applications. As a particularly advantageous mold oil composition, notation should be made of 80 a composition containing 90 to 98% of a reasonably good petroleum oil of say 40 viscosity, Saybolt, at 100° F., or of higher viscosity, and 10 to 2% of my addition material, which, as stated previously, is soluble in 85 petroleum oil. 90

I have found that this composition is non-gumming, does not oxidize in contact with air, and forms on the mold surface a tenaceous film which is not readily brushed, or 95 "washed", off by the flowing mix. Cutting oils may be improved by suitable additions,—up to say 50%,—of the said addition materials.

In the foregoing description mention has been made of the fact that my addition material is in part saponifiable and in part unsaponifiable. The saponifiable portion has been described as being a mixture of "acidic compounds" of high molecular weight. 100 While I have established definitely that said compounds have the nature and structure of saturated aliphatic hydroxycarboxylic acids, it is equally certain that said compounds in their normal state or when dissolved in petroleum or other non-aqueous solvent do not all react acid but are in part neutral in reaction. They, however, readily saponify with caustic alkali or alkali metal carbonate solutions,—especially upon heating 110 slightly,—to alkali metal salts of the simple acids. 115

These facts were brought out by the attempt to determine the molecular weights of these so-called "acids" by the freezing-point depression method, when it was found that the average molecular weight of the "acidic compounds" is approximately three times that of the molecule of average simple acid 125 as the latter is determined by titration, by 130

analysis of its silver salt, or by the Karl Rast method, using camphor as solvent. Be-  
richte, 1922, vol. 2, B, page 1051.

While I propose not to limit my invention  
5 by any hypothesis as to the actual chemical  
constitution of these acidic compounds, the  
results of my investigations to date would ap-  
pear to support the conception that they are  
10 rich in neutral-reacting esters, cyclic or ring  
esters, and inner-molecular anhydrides of  
simple aliphatic carboxylic acids of relatively  
high molecular weight, formed by the elimi-  
nation of water from one or more molecules  
15 of said simple acids.

15 This is indicated, for instance, when the  
simple acids (obtained by a careful acidification  
of their soap solution) are subjected to  
very careful drying at relatively low tem-  
perature; the molecular weights increase sub-  
stantially from 2 to 4 or more times those of  
the simple acids.

If the analogy between the simple acids of  
high molecular weight hereinbefore described  
and other better known and lower molecular  
25 weight simple saturated aliphatic carboxylic  
acids, e. g. lactic acid, is controlling, it would  
appear altogether probable that there occur  
condensations similar to those occurring in  
the cases of said simpler aliphatic oxy-car-  
30 boxylic acids, i. e., the formation of "double  
esters" (i. e., lactides), inner anhydrides (i. e.,  
lactones) and/or simple or complex esters  
(as, for example, by the combination of acids  
and alcohols or alcohol ketones present in  
35 the mixtures).

The following are suggestive representa-  
tions of some of the reactions thought to occur:



45 The above lactone formation is known to occur in my "addition materials", but whether it be  $\gamma$ , or  $\delta$  lactone is not known.



60 65 Such "ring esters" as the above lactide may

and probably do occur as three-, or four-  
membered rings.

The presence of such multi-membered  
rings has been demonstrated practically by  
substantially completely purifying the acidic 70  
compounds by separating them from the  
naturally associated ketones, alcohols, keto-  
alcohols and alcohol-ketones by extraction  
with ether, and determining their average  
molecular weight by the freezing-point de- 75  
pression method. The average molecular  
weight (less the water eliminated by slight  
heating) is approximately three times the  
average molecular weight of the acids them-  
selves as found by the silver salt analysis 80  
or direct titration methods. From this find-  
ing, and from the fact that lactones, of the  
above character occur in said mixtures, I de-  
duce that said mixtures contain condensation  
products ranging from lactones up to say 85  
six-membered "ring esters", with an average  
of three-membered ring esters.

I claim:

1. The method of increasing the lubricat-  
ing properties of an oil of petroleum origin 90  
which consists in adding to said oil an oil-  
soluble addition material obtainable by ox-  
idizing a mixture consisting essentially of  
relatively high molecular-weight, saturated,  
aliphatic hydrocarbons of mineral origin, in 95  
the liquid phase, at a temperature of from  
about 100° to about 150° C. and at a super-  
atmospheric pressure not greater than about  
320 pounds per square inch, in the presence  
of an exciter of oxidation, until the point of 100  
incipient formation of compounds which are  
insoluble in petroleum and in the reaction  
mixture, which mixture comprises saponifi-  
able and unsaponifiable components, separat-  
ing the saponifiable components from at least 105  
the major portion of the unsaponifiable com-  
ponents, treating the separated portion con-  
taining said saponifiable components with  
steam until substantially no more volatile  
material passes over, and drying the result- 110  
ing residue.

2. The method of increasing the lubricat-  
ing properties of an oil of petroleum origin 115  
which consists in adding to said oil an oil-  
soluble addition material obtainable by ox-  
idizing a mixture consisting essentially of  
relatively high molecular-weight, saturated,  
aliphatic hydrocarbons of mineral origin, in 120  
the liquid phase, at a temperature of from  
about 100° to about 150° C. and at a super-at-  
mospheric pressure not greater than about  
320 pounds per square inch, in the presence  
of an exciter of oxidation, until the point of 125  
incipient formation of compounds which are  
insoluble in petroleum and in the reaction  
mixture, treating the resulting reaction mix-  
ture with hot aqueous solution of caustic  
alkali, separating the resulting soap solution  
from unsaponifiable components of the reac- 130  
tion mixture and diluting said soap solution 135

with water until the solution becomes clear, acidifying the solution, separating the resulting precipitate, treating the precipitate with steam until substantially no more volatile material passes over, and drying the resulting residue.

3. The method of increasing the lubricating properties of an oil of petroleum origin which consists in adding to said oil an oil-soluble addition material obtainable by oxidizing a mixture consisting essentially of relatively high molecular-weight, saturated, aliphatic hydrocarbons of mineral origin, in the liquid phase, at a temperature of from about 100° to about 150° C. and at a super-atmospheric pressure not greater than about 320 pounds per square inch, in the presence of an exciter of oxidation, until the point of incipient formation of compounds which are insoluble in petroleum and in the reaction mixture, treating the resulting reaction mixture with hot aqueous solution of caustic alkali, separating the resulting soap solution from unsaponifiable components of the reaction mixture and diluting said soap solution with water until the solution becomes clear, acidifying the solution, separating the resulting precipitate, treating the precipitate with steam until substantially no more volatile material passes over, and drying the resulting residue.

10 4. The method of increasing the lubricating properties of an oil of petroleum origin which consists in adding to said oil an oil-soluble addition material of mineral origin, said addition material being substantially free of hydrocarbons and consisting essentially of high-molecular-weight aliphatic oxygen-containing compounds including a substantial proportion of free saturated aliphatic carboxylic acids.

40 5. As a new product adapted for use in admixture with a lubricating oil of petroleum origin, an oil-soluble addition material obtainable by oxidizing a mixture consisting essentially of relatively high molecular-weight, saturated, aliphatic hydrocarbons of mineral origin, in the liquid phase, at a temperature of from about 100° to about 150° C. and at a super-atmospheric pressure not greater than about 320 pounds per square inch, in the presence of an exciter of oxidation, until the point of incipient formation of compounds which are insoluble in petroleum and in the reaction mixture, which mixture comprises saponifiable and unsaponifiable components, separating the saponifiable components from at least the major portion of the unsaponifiable components, treating the separated portion containing said saponifiable components with steam until substantially no more volatile material passes over, and drying the resulting residue.

60 6. As a new product adapted for use in admixture with a lubricating oil of petroleum origin, an oil-soluble addition material obtainable by oxidizing a mixture consisting es-

entially of relatively high molecular-weight, saturated, aliphatic hydrocarbons of mineral origin, in the liquid phase, at a temperature of from about 100° to about 150° C. and at a super-atmospheric pressure not greater than 70 about 320 pounds per square inch, in the presence of an exciter of oxidation, until the point of incipient formation of compounds which are insoluble in petroleum and in the reaction mixture, treating the resulting reaction mixture with hot aqueous solution of caustic alkali, separating the resulting soap solution from unsaponifiable components of the reaction mixture and diluting said soap solution with water until the solution becomes clear, acidifying the solution, separating the resulting precipitate, treating the precipitate with steam until substantially no more volatile material passes over, and drying the resulting residue.

75 7. As a new product adapted for use in admixture with a lubricating oil of petroleum origin, an oil-soluble addition material obtainable by oxidizing a mixture consisting essentially of relatively high molecular-weight, 80 saturated, aliphatic hydrocarbons of mineral origin, in the liquid phase, at a temperature of from about 100° to about 150° C. and at a super-atmospheric pressure not greater than about 320 pounds per square inch, in the presence of an exciter of oxidation, until the point of incipient formation of compounds which are insoluble in petroleum and in the reaction mixture, which mixture comprises 85 saponifiable and unsaponifiable components, extracting the said mixture with an organic solvent for the saponifiable components, separating the organic solvent from the so-separated portion of the reaction mixture, treating the said portion with steam until substantially no more volatile material passes over, and drying the resulting residue.

90 8. As a new product adapted for use in admixture with a lubricating oil of petroleum origin, an oil-soluble addition material of 100 mineral origin, said addition material being substantially free of hydrocarbons and consisting essentially of high-molecular-weight aliphatic oxygen-containing compounds including a substantial proportion of free saturated aliphatic carboxylic acids.

105 9. The method of increasing the lubricating properties of an oil which consists in adding to said oil an oil-soluble addition material of mineral origin consisting of free saturated aliphatic carboxylic acids from about 110 23% to about 40% by weight, neutral lactones and esters derived from said acids from about 7% to about 50%, and unsaponifiable non-acidic, oxygen-containing aliphatic compounds from about 25% to about 40%.

115 10. A composition of matter consisting of lubricating oil of petroleum origin and an oil-soluble addition material obtainable by oxidizing a mixture consisting essentially of

- relatively high molecular-weight, saturated, aliphatic hydrocarbons of mineral origin, in the liquid phase, at a temperature of from about 100° to about 150° C. and at a super-atmospheric pressure not greater than about 320 pounds per square inch, in the presence of an exciter of oxidation, until the point of incipient formation of compounds which are insoluble in petroleum and in the reaction mixture, which mixture comprises saponifiable and unsaponifiable components, separating the saponifiable components from at least the major portion of the unsaponifiable components, treating the separated portion containing said saponifiable components with steam until substantially no more volatile material passes over, and drying the resulting residue. 11. A composition of matter consisting of lubricating oil of petroleum origin and an oil-soluble addition material obtainable by oxidizing a mixture consisting essentially of relatively high molecular-weight, saturated, aliphatic hydrocarbons of mineral origin, in the liquid phase, at a temperature from about 100° to about 150° C. and at a super-atmospheric pressure not greater than about 320 pounds per square inch, in the presence of an exciter of oxidation, until the point of incipient formation of compounds which are insoluble in petroleum and in the reaction mixture, treating the resulting reaction mixture with hot aqueous solution of caustic alkali, separating the resulting soap solution from unsaponifiable components of the reaction mixture and diluting said soap solution with water until the solution becomes clear, acidifying the solution, separating the resulting precipitate, treating the precipitate with steam until substantially no more volatile material passes over, and drying the resulting residue. 12. A composition of matter consisting of lubricating oil of petroleum origin and an oil-soluble addition material obtainable by oxidizing a mixture consisting essentially of relatively high molecular-weight, saturated, aliphatic hydrocarbons of mineral origin, in the liquid phase, at a temperature of from about 100° to about 150° C. and at a super-atmospheric pressure not greater than about 320 pounds per square inch, in the presence of an exciter of oxidation, until the point of incipient formation of compounds which are insoluble in petroleum and in the reaction mixture, which mixture comprises saponifiable and unsaponifiable components, extracting the said mixture with an organic solvent for the saponifiable components, separating the organic solvent from the so-separated portion of the reaction mixture, treating the said portion with steam until substantially no more volatile material passes over and drying the resulting residue. 13. A composition of matter consisting of lubricating oil of petroleum origin and an oil-soluble addition material of mineral origin, said addition material being substantially free of hydrocarbons and consisting essentially of high-molecular-weight aliphatic oxygen-containing compounds including a substantial proportion of free saturated aliphatic carboxylic acids. 14. A composition of matter consisting of lubricating oil of petroleum and an oil-soluble addition material of mineral origin consisting of free saturated aliphatic carboxylic acids from about 23% to about 40% by weight, neutral lactones and esters derived from said acids from about 7% to about 50%, and unsaponifiable non-acidic, oxygen-containing aliphatic compounds from about 25% to about 40%. 15. A composition of matter consisting of from about 90.0% to about 99.75% by weight of lubricating oil of petroleum origin and from about 10.0% to about 0.25% by weight of an oil-soluble addition material obtainable by oxidizing a mixture consisting essentially of relatively high molecular-weight, saturated, aliphatic hydrocarbons of mineral origin, in the liquid phase, at a temperature of from about 100° to about 150° C. and at a super-atmospheric pressure not greater than about 320 pounds per square inch, in the presence of an exciter of oxidation, until the point of incipient formation of compounds which are insoluble in petroleum and in the reaction mixture, which mixture comprises saponifiable and unsaponifiable components, separating the saponifiable components from at least the major portion of the unsaponifiable components, treating the separated portion containing said saponifiable components with steam until substantially no more volatile material passes over, and drying the resulting residue. 16. A composition of matter consisting of from about 90.0% to about 99.75% by weight of lubricating oil of petroleum origin and from about 10.0% to about 0.25% by weight of an oil-soluble addition material obtainable by oxidizing a mixture consisting essentially of relatively high molecular-weight, saturated, aliphatic hydrocarbons of mineral origin, in the liquid phase, at a temperature of from about 100° to about 150° C. and at a super-atmospheric pressure not greater than about 320 pounds per square inch, in the presence of an exciter of oxidation, until the point of incipient formation of compounds which are insoluble in petroleum and in the reaction mixture, treating the resulting reaction mixture with hot aqueous solution of caustic alkali, separating the resulting soap solution from unsaponifiable components of the reaction mixture and diluting said soap solution with water until the solution becomes clear, acidifying the solution, separating the resulting precipitate, treating the precipitate with

steam until substantially no more volatile material passes over, and drying the resulting residue.

17. A composition of matter consisting of  
5 from about 90.0% to about 99.75% by weight  
of lubricating oil of petroleum origin and  
from about 10.0% to about 0.25% by weight  
of an oil-soluble addition material obtainable  
10 by oxidizing a mixture consisting essentially  
of relatively high molecular-weight, satu-  
rated, aliphatic hydrocarbons of mineral  
origin, in the liquid phase, at a temperature  
of from about 100° to about 150° C. and at  
a super-atmospheric pressure not greater than  
15 about 320 pounds per square inch, in the pres-  
ence of an exciter of oxidation, until the point  
of incipient formation of compounds which  
are insoluble in petroleum and in the reaction  
mixture, which mixture comprises saponifi-  
20 able and unsaponifiable components, extract-  
ing the said mixture with an organic solvent  
for the saponifiable components, separating  
the organic solvent from the so-separated por-  
tion of the reaction mixture, treating the said  
25 portion with steam until substantially no  
more volatile material passes over and drying  
the resulting residue.

18. A composition of matter consisting of  
from about 90.0% to about 99.75% by weight  
30 of lubricating oil of petroleum origin and  
from about 10.0% to about 0.25% by weight  
of an oil-soluble material of mineral origin,  
said addition material being substantially  
35 free of hydrocarbons and consisting essen-  
tially of high-molecular-weight aliphatic  
oxygen-containing compounds including a  
substantial proportion of free saturated ali-  
phatic carboxylic acids.

In testimony whereof, I affix my signature.  
ARTHUR W. BURWELL.

40

45

50

55

60

65